

July 21, 1964

B. DAVIES ET AL

3,141,790

BURNED BASIC REFRACTORY SHAPES

Filed Jan. 25, 1963



*Fig. 2*



*Fig. 1*

INVENTORS:

BEN DAVIES  
ERNEST PAUL WEAVER  
PETER HARRY HAVRANEK  
BY *William C. Neal*  
ATTORNEY

## 1

3,141,790

### BURNED BASIC REFRACtORY SHAPES

Ben Davies, Ernest Paul Weaver, and Peter Harry Havranek, Pittsburgh, Pa., assignors to Harbison-Walker Refractories Company, Pittsburgh, Pa., a corporation of Pennsylvania

Filed Jan. 25, 1963, Ser. No. 254,013

9 Claims. (Cl. 117—123)

This invention relates to furnace structure for the oxygen steelmaking process. More particularly, this invention relates to the working lining of oxygen steelmaking vessels.

In the oxygen steelmaking processes, which have been variously designated as the "LD" process, basic oxygen furnace process, oxygen converter process, etc., the furnace structure normally consists of a metal shell having a refractory lining therein. The lining for oxygen vessels has heretofore generally consisted of an inner or "working" lining of tar bonded, chemically bonded, or burned basic brick, an exterior or shell lining of burned magnesite brick, and usually an intermediate layer of a tar bonded ramming mix of composition similar to that of the working lining. This invention is primarily concerned with the working lining, and a composition suitable for use therein. In a particular aspect, the invention relates to improved lining material for the cone section and a slag splash zone of an oxygen converter lining.

Refractory shapes may be termed chemically bonded or ceramically bonded. The chemically bonded shapes are green or unfired shapes, and are put into service in this form. Ceramically bonded shapes are shapes which have been subjected to elevated burning or firing temperatures, to obtain a ceramic bond throughout the particulate material from which the shape is fabricated. This invention relates particularly to the latter.

In both chemically and ceramically bonded shapes, the bond itself is probably one of the most important properties. In order to obtain a shape which is easily handled and which stands up in service without spalling, peeling or breaking away, the bond must be strong and relatively stable. For certain uses, high density and low porosity are equally important properties. These latter properties are desirable in a shape, to resist penetration by corrosive metallurgical slags and fumes which tend to destroy a shape in service.

Typically, the lining of an oxygen converter has been made of basic refractories, because the slag of the oxygen steelmaking process is, itself, basic. Prior refractories most commonly used are those consisting essentially of tar impregnated or tar bonded, dead burned magnesite, dead burned dolomite, and sometimes lime mixed with the foregoing. Since this invention relates particularly to burned or ceramically bonded shapes, it is most closely related to the art of tar impregnated basic refractories. An example of a good tar impregnated dead burned magnesite refractory is one made according to the teachings of United States application, Serial No. 113,094, Davies et al., filed May 29, 1961, entitled "Burned Refractory Product," now United States Patent No. 3,106,475, and owned by the same assignee as the instant invention. The shapes of the invention of the co-pending application are particularly adapted to manufacture by conventional techniques using commercially

## 2

available materials. One of their outstanding properties is resistance to impact, abrasion and spalling. These brick are characterized by good strength at room temperature and by very good compressive strength at elevated temperatures, as indicated by resistance to subsidence in a load test at elevated temperatures. However, in service, ceramically bonded brick are subjected to tensile stress due to expansion and the like. And, while the refractories of application Serial No. 113,094 have high compressive strength, they do not resist tensile stresses as much as might be desired.

Accordingly, it is an object of this invention to provide ceramically bonded shapes having improved tensile strength, particularly suited for use in fabrication of the lining of oxygen converter vessels.

It is another object of this invention to provide refractory shapes having improved resistance to tensile stresses in service installations.

In one aspect, this invention is predicated on the discovery that controlled adulteration of very high purity dead burned magnesia grain (i.e., 97+% MgO, by weight, and on the basis of an oxide analysis) and use of this grain in the manufacture of a ceramically bonded shape with subsequent tar impregnation thereof, provides shapes giving superior service in an oxygen converter vessel. The  $R_2O_3$  content of the grain and the resulting shapes is critical. We have found it must be less than about 1%, by weight, of the grain. As known to those in the art, " $R_2O_3$ " refers to  $Cr_2O_3$ ,  $Fe_2O_3$  and  $Al_2O_3$ . Our so-called adulterating ingredients are lime and silica. The silica must constitute less than about 1% of the grain and shapes, with at least 3 but not more than 4 times as much lime as silica expressed as  $CaO$  and  $SiO_2$ .

A better understanding and other features and advantages of our invention will become obvious to those skilled in the metallurgical and refractory arts, by a reading of the following detailed description with reference to specific examples and to the drawings. In these drawings:

FIG. 1 is a photomicrograph of a portion of a ceramically bonded shape according to this invention; and

FIG. 2 is a photomicrograph of a previous ceramically bonded shape.

Workers in the art of refractories and related ceramic fields have long recognized that lime and silica can be balanced in a basic refractory, i.e. one fabricated of a magnesite or a dolomite, to good advantage. The United States Patent to Pitt, No. 2,245,297, the Patent to McCaughey et al., No. 1,965,605, the Patent to Lee, No. 2,089,970, the Patent to Lee, No. 2,229,297, and others, are all indicative of prior work in this area. The basic goal of these workers appears to have been stabilization of the materials with which they worked (especially the lime). Also, they reported desirable improvement in various physical properties, including strength.

The ceramically bonded shapes according to the co-pending application, Serial No. 113,094, mentioned above, on infrequent occasion exhibit a distressing loss of strength at temperatures above 2000° F. This loss of hot strength is believed to be caused by the weakening of the very thin silicate films that appear to coat and bond the separate magnesia or periclase crystals which constitute the shapes. FIG. 2 is a photomicrograph (1000 $\times$  magnification) of a shape according to the co-pending ap-

plication, in which periclase crystals 10 are shown cemented in place and largely surrounded by monticellite 11 and merwinite 12 (both silicate minerals) films. The numeral 13 indicates voids.

More recently, we have come to realize that to develop the best tensile strength in a magnesite brick, there must be a direct attachment of magnesite or periclase crystal to periclase crystal without an intervening film of silicate.

In order to achieve this direct attachment, we made brick from the most pure commercially available refractory magnesite of which we know, having the analysis of grain AA shown in Table I, using conventional brick-making and burning temperatures. Upon testing these brick for modulus of rupture at 2300° F., we found they were no stronger than those made of lower purity magnesite. Petrographic examination revealed that a silicate film still separated most of the separate magnesia or periclase crystals (similar to the showing of FIG. 2). In attempting to overcome this problem, we burned similar refractory shapes to a temperature of 3400° F. which far exceeds any commercial burning practice but this did not remove the silicate film nor improve the strength at 2300° F.

It became apparent that no physical processing was likely to remove this silicate film, because the lowest surface energy for the system was still a magnesium silicate-magnesia bond, rather than the desired magnesia-magnesia bond.

The studies of prior workers, such as those of the United States patents, above noted, and our own work, suggested that conversion of these silicate films to a dicalcium silicate would be useful.

In exploratory studies, we prepared a size graded batch of dead burned magnesite, to which we added a small amount of lime hydrate and a small amount of chromic oxide to stabilize any dicalcium silicate against mineral inversion, if this silicate should form in burning. The magnesite used had the following chemical analysis.

Table I

## Grain AA:

|                                      |         |        |
|--------------------------------------|---------|--------|
| SiO <sub>2</sub> -----               | percent | 0.9    |
| Al <sub>2</sub> O <sub>3</sub> ----- | do      | 0.4    |
| Fe <sub>2</sub> O <sub>3</sub> ----- | do      | 0.3    |
| CaO -----                            | do      | 1.1    |
| MgO -----                            | do      | 97.3   |
| Ratio CaO/SiO <sub>2</sub> -----     |         | 1.22/1 |

All parts by weight, and on the basis of an oxide analysis.

The size grading of the magnesite grain was substantially as follows:

Table II

|                             | Percent |
|-----------------------------|---------|
| -4 on 10 mesh               | 40      |
| -10 on 28 mesh              | 15      |
| -28 on 65 mesh              | 15      |
| -65 mesh to ball mill fines | 30      |

To about 98.5 parts of the magnesite, size graded as indicated, we added 1.3 parts of lime hydrate (technical grade) and about 0.2 part chromic oxide (also technical grade). These materials were dry mixed for about five minutes and then for an additional five minutes while adding 2 parts lignin liquor and 2 parts water, based on the total weight of the mixture, as a tempering fluid. Brick were made from the batch by pressing on a power press at 8000 p.s.i. and burned 4 high on edge to cone 23 (about 2820° F.). These brick were subjected to physical testing, the results of which are set forth in Table III.

Table III

|                                     |         |      |
|-------------------------------------|---------|------|
| Linear change in burning -----      | percent | -0.1 |
| Bulk density, p.c.f. (av. 20) ----- | do      | 174  |
| Modulus of rupture, p.s.i. (av. 3): |         |      |
| At room temperature -----           |         | 1360 |
| At 1500° F. (5 hr. hold) -----      |         | 930  |
| At 2000° F. (5 hr. hold) -----      |         | 870  |
| At 2300° F. (5 hr. hold) -----      |         | 400  |
| Apparent porosity (av. 5) -----     | percent | 20.1 |

Comparative batches of the same magnesite without the lime hydrate or chromic oxide additions are mixes A through D of Table V. The lime hydrate addition of the Table III mix obviously improved the tensile strength at elevated temperatures. This is readily apparent from comparing the modulus of rupture at 2300° F. for Table III with mixes A through D of Table V, which contained no added lime hydrate. However, the increased strength was still less than that desired. Microscopic studies of brick made from the mix to which the lime hydrate had been added still indicated a silicate filming, somewhat similar to that previously observed with brick of the type shown in FIG. 2 of the drawings.

We therefore concluded, that to change the characteristics of this system some additive had to be made to the brick mix. Thus, to brick batch mixtures of the type described in Tables I and II, 1% of the following oxides were added: Al<sub>2</sub>O<sub>3</sub>, Cr<sub>2</sub>O<sub>3</sub>, Fe<sub>2</sub>O<sub>3</sub>, NiO, CaO, ZnO, CuO, TiO<sub>2</sub> (all technical grade and -325 mesh). Brick were pressed from these batches and burned at cone 23 (some of this work is reported in more detail below). None of these additions had any appreciable effect on the strength at 2300° F.

It was then decided to more fully explore the field of controlled lime additions to the magnesite grain-making batch, with attention to the relationship of lime content to the other oxides. We prepared an extended series of these magnesites, and one which proved to have extremely interesting properties was the grain BB of Table IV. It was made by utilizing the same magnesium hydroxide slurry, which was the initial ingredient of grain AA. Additions of lime hydrate were made which, after caustic burning, gave an analysis typically as follows.

Table IV

## Grain BB:

|                                      |         |        |
|--------------------------------------|---------|--------|
| MgO -----                            | percent | 96.3   |
| SiO <sub>2</sub> -----               | do      | 0.8    |
| CaO -----                            | do      | 2.9    |
| Fe <sub>2</sub> O <sub>3</sub> ----- | do      | 0.3    |
| Al <sub>2</sub> O <sub>3</sub> ----- | do      | 0.4    |
| Ratio CaO/SiO <sub>2</sub> -----     |         | 3.63/1 |

This caustic calcined mixture, with all free and substantially all chemically combined water removed, was formed into small briquettes at a pressure of about 20,000 p.s.i., which briquettes were fed to a shaft kiln where they were dead burned at a temperature above about 3000° F. The resulting dead burned briquettes were crushed to formulate brickmaking grain. This grain, whose analysis is typified by Table IV, was then used for fabrication of various brickmaking batches, as reported in Table V, mixes E, F, G and H. These batches were subjected to brick fabricating and burning techniques, substantially the same as described above, with reference to Table I. Table V sets forth in detail the composition of the various batches and the results of physical testing of brick made from the batches. The abbreviation BMF refers to ball milled fines. The brick were burned to cone 23 (2820° F.) with the top temperature being held for 10 hours.

Table V

| Magnesite Grain.....                                              | 100% Grain AA |        |        |        | 100% Grain BB<br>(Co-burned with CaO) |        |        |        | Grain<br>AA but<br>with<br>BB in<br>BMF | Grain<br>BB but<br>with<br>AA in<br>BMF |
|-------------------------------------------------------------------|---------------|--------|--------|--------|---------------------------------------|--------|--------|--------|-----------------------------------------|-----------------------------------------|
|                                                                   | A             | B      | C      | D      | E                                     | F      | G      | H      |                                         |                                         |
| Mix Letter.....                                                   |               |        |        |        |                                       |        |        |        |                                         |                                         |
| Batch:                                                            |               |        |        |        |                                       |        |        |        |                                         |                                         |
| -3+10 mesh.....                                                   |               | 20     | 30     | 40     |                                       | 20     | 30     | 40     |                                         |                                         |
| -4+10 mesh.....                                                   | 34            | 20     | 10     |        | 34                                    | 20     | 10     |        | 34                                      | 34                                      |
| -10+28 mesh.....                                                  | 28            | 20     | 20     | 20     | 28                                    | 20     | 20     | 20     | 28                                      | 28                                      |
| BMF (50-60% -325 mesh).....                                       | 38            | 40     | 40     | 40     | 38                                    | 40     | 40     | 40     | 38                                      | 38                                      |
| Lignin Liquor and water, about 50/50<br>weight ratio percent..... | 5             | 5      | 5      | 5      | 5                                     | 5      | 5      | 5      | 5                                       | 5                                       |
| Bulk Density, p.c.f. (Av. 10).....                                | 180           | 181    | 181    | 182    | 180                                   | 181    | 181    | 182    | 178                                     | 180                                     |
| Modulus of Rupture, p.s.i.:                                       |               |        |        |        |                                       |        |        |        |                                         |                                         |
| At Room Temperature, about 72° F.<br>(Av. 3).....                 | 2,450         | 2,370  | 2,190  | 2,200  | 2,150                                 | 2,570  | 2,740  | 2,760  | 2,150                                   | 2,360                                   |
| At 2300° F. (Hold Time 5 Hours Av. 3).....                        | 180           | 140    | 130    | 120    | 1040                                  | 920    | 990    | 985    | 500                                     | 860                                     |
| Chemical Analysis of Batch:                                       |               |        |        |        |                                       |        |        |        |                                         |                                         |
| Silica (SiO <sub>2</sub> ).....percent.....                       | 0.8           | 0.8    | 0.8    | 0.8    | 0.8                                   | 0.8    | 0.8    | 0.8    | 0.8                                     | 0.8                                     |
| Lime (CaO).....do.....                                            | 0.9           | 0.9    | 0.9    | 0.9    | 2.9                                   | 2.9    | 2.9    | 2.9    | 1.7                                     | 2.1                                     |
| Lime/Silica Ratio.....do.....                                     | 1.13/1        | 1.13/1 | 1.13/1 | 1.13/1 | 3.62/1                                | 3.62/1 | 3.62/1 | 3.62/1 | 2.13/1                                  | 2.63/1                                  |

The results of the testing reported in Table V were completely unexpected. The brick fabricated entirely from the special co-burned grain (mixes E through H) had a modulus of rupture at 2300° F. over 4 and almost 5 times as great as the comparative samples (A through D) not having the benefit of the lime addition before dead burning of the magnesia. Mixes I and J indicated beneficial characteristics were imparted when even a portion of the batch was fabricated of the co-burned grain with a carefully balanced lime/silica ratio, with best results obtained when the special grain was included as the coarse fraction (mix J).

Microscopic examination of the brick fabricated entirely from the special co-burned grain revealed a dramatic change in appearance as compared to previous ceramically bonded brick of this type, as typified by FIG. 2 (1000 $\times$  magnification). FIG. 1 is a photomicrograph of a brick fabricated entirely of the special co-burned grain (1000 $\times$  magnification). These latter brick are characterized by direct periclase to periclase crystal or grain attachment. In FIG. 1, the large white areas are the periclase grains. The lime and silica appear to collect in small, generally diamond-shaped pools or deposits 16. X-ray analysis showed these deposits to be substantially all tricalcium silicate. The irregular areas 17 are voids.

The results of Table V are even more surprising when compared to the results of Table III above, in which lime hydrate was added to a size graded dead burned magnesite batch to provide an overall lime/silica ratio of about 2 in the batch. In further studies, co-burned grain was manufactured, in which the lime/silica ratio was about 4.16 to 1. Under identical testing conditions, it was found that a lime/silica ratio of this magnitude and slightly higher is satisfactory, but such ratios undesirably complicate manufacturing. Also greater amounts of lime increase the hydration tendency of shapes made from such grain. The entire series of tests established to our satisfaction that the optimum range for the lime/silica ratio should be between 3 to 1 and 4 to 1. The 4 to 1 ratio is somewhat flexible, with satisfactory product resulting with a ratio as high as 4.5 to 1.

Since the pooling of the silicate was so unexpected and different from the previous silicate filming we had observed, it appeared likely the presence of other oxides in the brick mix might affect the silicate surface tension and give still better properties to the brick.

For example, we expected that a small amount of chromic oxide, such as that added to the batch which included the lime hydrate reported in Table III, would provide even greater strength for shapes according to this invention. We, therefore, prepared another batch

of the co-burned grain, having a balanced lime/silica ratio of 3.62:1. The batch was substantially the same as mix E of Table V. We added 1%, by weight, of technical grade chromic oxide (all -325 mesh) to the batch, and manufactured it into brick according to the same techniques discussed with reference to Table III above. The resulting burned brick had a modulus of rupture at 2300 of only 390 p.s.i. This indicated that R<sub>2</sub>O<sub>3</sub> type materials might generally have a detrimental effect on the brick of our invention. We, therefore, prepared two additional batches of the same grain, and having the same size grading, to the first of which we added Al<sub>2</sub>O<sub>3</sub> (technical grade alumina) to total about 1% for the batch, and to the second of which we added Fe<sub>2</sub>O<sub>3</sub> (pigment grade iron oxide) to total about 1% of the batch. Brick fabricated of the batch having the alumina addition had a modulus of rupture of 280 p.s.i. at 2300° F. Brick made from the batch with the iron oxide addition had a somewhat higher modulus of rupture at 2300° F.; namely, 410 p.s.i. We, therefore, concluded that the total amount of R<sub>2</sub>O<sub>3</sub> materials in the grain and brick must be maintained at a level below 1%, by weight.

In our extensive work in the field of this invention, we sometimes find that if all of the other factors are suitably confined, control of the ratio of CaO to SiO<sub>2</sub> is an adaptable device for maintaining product quality. At the same time, when we so operate that the CaO/SiO<sub>2</sub> ratio is between 3/1 and 4/1, we are, in effect, making sure that the principal non-magnesia crystalline ingredient is tricalcium silicate (3CaO·SiO<sub>2</sub>). This may at first appear puzzling since, on a molecular basis, this mineral contains CaO and SiO<sub>2</sub> in the ratio of only 2.8/1.

In working in this field, we find it convenient to appraise our mixes in terms of the ratio of CaO to SiO<sub>2</sub> of the various compositions. If a magnesite should be made available, in which all of the CaO and SiO<sub>2</sub> were present as dicalcium silicate (2CaO·SiO<sub>2</sub>), the CaO/SiO<sub>2</sub> ratio would be 1.87/1, which is calculated from the molecular weights; if present solely as tricalcium silicate



the CaO/SiO<sub>2</sub> ratio would be 2.8/1; if present solely as wollastonite (CaO·SiO<sub>2</sub>), the CaO/SiO<sub>2</sub> ratio would be 0.93. If a magnesite should contain more CaO than the 2.8/1 ratio of tricalcium silicate, the excess CaO would necessarily be present as some mineral other than calcium silicates, since there is no calcium silicate more calcareous than tricalcium silicate. Such excess CaO is thought of as existing as ferrites, or aluminates (if the requisite Fe<sub>2</sub>O<sub>3</sub> and Al<sub>2</sub>O<sub>3</sub> are present) or as free lime.

The co-burned grain BB of Table IV is illustrative. Its CaO/SiO<sub>2</sub> ratio was 3.63/1, which is considerably above the 2.8/1 of tricalcium silicate. Nevertheless, in the microscopic examinations no silicate other than tricalcium silicate and free CaO was unobserved. In our experience, as we proceed upwards to the neighborhood of 4/1 ratios, free lime can be expected to make its appearance. A small amount can be tolerated but, for reasons mentioned elsewhere, free lime in the grain or finished brick introduces difficulties, which can become prohibitive in nature.

The foregoing discussion of experimental data, demonstrates the superiority in physical properties and, in particular, the superiority in hot strength as measured by modulus of rupture at 2300° F., for brick made in accordance with our invention. We also demonstrated that they exhibited adequate resistance to thermal shock, as evidenced by 0.0% spalling loss when subjected to ASTM C-122 thermal shock tests. The combination of thermal shock resistance and hot strength renders them particularly suitable in locations in an oxygen process vessel, where mechanical wear and rapid temperature changes are present; namely, in the cone and slag splash zones of oxygen converter vessels. Of course, they are tar impregnated for use in these vessels. We suggest between 4 and 10%, by weight, of tar in the brick as being most suitable. Between 6 and 8% tar is best.

A group of burned brick, fabricated according to this invention, are giving outstanding service in oxygen converter vessels. The brick are impregnated with cokable, non-aqueous, carbonaceous materials such as tar and pitch. They were impregnated by immersion in the carbonaceous material, generally heated to about 400° F.

The heated and liquified carbonaceous material easily penetrates throughout the brick and, in cross section, the brick show remarkably uniform distribution of the carbonaceous material, including a thin layer completely about exterior surfaces. Commercially available tar or pitch of petroleum or coal base can be used for impregnation. Generally, we suggest a coal based pitch, having a softening point on the order of 150° F.

Unless otherwise stated, all chemical analyses are on the basis of an oxide analysis, in conformity with the common practice of reporting the chemical analyses of refractory materials. All size grading is according to the Tyler mesh series. All parts and percentages are by weight. The chemical analyses of raw materials, which are reported, should be considered typical. However, the lime, silica and R<sub>2</sub>O<sub>3</sub> content, reported in the various analyses, should be considered accurate to the first decimal place.

Having thus described the invention in detail and with sufficient particularity as to enable those skilled in the art to practice it, what is desired to have protected by Letters Patent is set forth in the following claims.

We claim:

1. Tar impregnated, ceramically bonded basic refractory shapes suitable for use in metallurgical vessels, said shapes, by weight and on the basis of an oxide analysis, consisting essentially of from about 96 to 97% MgO, there being CaO and SiO<sub>2</sub> in a weight ratio between 3 to 1 and about 4 to 1, and materials of the group Cr<sub>2</sub>O<sub>3</sub>, Al<sub>2</sub>O<sub>3</sub>, and Fe<sub>2</sub>O<sub>3</sub>, in an amount not exceeding 1%, said shapes microscopically characterized by periclase to periclase crystal attachment and with the CaO and SiO<sub>2</sub> content largely present in spaced disconnected pockets between the periclase crystals and being mineralogically characterized largely as tricalcium silicate.

2. Tar impregnated ceramically bonded basic refractory shapes suitable for use in metallurgical vessels, said shapes made from a batch of size graded dead burned magnesia grain, at least a portion of the grain by weight and on the basis of an oxide analysis, consisting essentially

of from about 96 to 97% MgO, there being CaO and SiO<sub>2</sub> in a weight ratio between 3 to 1 and about 4 to 1, and materials of the group Cr<sub>2</sub>O<sub>3</sub>, Al<sub>2</sub>O<sub>3</sub> and Fe<sub>2</sub>O<sub>3</sub>, in an amount not exceeding 1%, and being made by co-burning the MgO, CaO and SiO<sub>2</sub> ingredients thereof.

3. Ceramically bonded basic refractory shapes suitable for use in metallurgical vessels, said shapes, by weight and on the basis of an oxide analysis, consisting essentially of from about 96 to 97% MgO, there being CaO and SiO<sub>2</sub> in a weight ratio between 3 to 1 and about 4 to 1, and materials of the group Cr<sub>2</sub>O<sub>3</sub>, Al<sub>2</sub>O<sub>3</sub>, and Fe<sub>2</sub>O<sub>3</sub>, in an amount not exceeding 1%, said shapes microscopically characterized by periclase to periclase crystal attachment and with the CaO and SiO<sub>2</sub> content largely present in spaced disconnected pockets between the periclase crystals and being mineralogically characterized largely as tricalcium silicate.

4. Ceramically bonded basic refractory shapes suitable for use in metallurgical vessels, said shapes made from a batch of size graded dead burned magnesia grain, at least a portion of the grain by weight and on the basis of an oxide analysis, consisting essentially of from about 96 to about 97% MgO, there being CaO and SiO<sub>2</sub> in a weight ratio between 3 to 1 and about 4 to 1, and materials of the group Cr<sub>2</sub>O<sub>3</sub>, Al<sub>2</sub>O<sub>3</sub>, and Fe<sub>2</sub>O<sub>3</sub>, in an amount not exceeding 1%, and being made by co-burning the MgO, CaO and SiO<sub>2</sub> ingredients thereof.

5. Tar impregnated, ceramically bonded basic refractory shapes suitable for use in metallurgical vessels, said shapes, by weight and on the basis of an oxide analysis, consisting essentially of from about 0.8 to no more than about 1% SiO<sub>2</sub>, CaO in an amount sufficient to obtain a CaO to SiO<sub>2</sub> weight ratio between about 3 to 1 and about 4 to 1, the remainder consisting essentially of MgO and materials of the group Fe<sub>2</sub>O<sub>3</sub>, Cr<sub>2</sub>O<sub>3</sub>, and Al<sub>2</sub>O<sub>3</sub>, said latter materials constituting less than about 1% of the total weight of the batch.

6. Tar impregnated ceramically bonded basic refractory shapes suitable for use in metallurgical vessels, said shapes made from a batch of size graded dead burned magnesia grain, at least a portion of the grain, by weight and on the basis of an oxide analysis, consisting essentially of from about 0.8 to no more than about 1% SiO<sub>2</sub>, CaO in an amount sufficient to obtain a CaO to SiO<sub>2</sub> weight ratio between about 3 to 1 and about 4 to 1, the remainder consisting essentially of MgO and materials of the group Fe<sub>2</sub>O<sub>3</sub>, Cr<sub>2</sub>O<sub>3</sub>, and Al<sub>2</sub>O<sub>3</sub>, said latter materials constituting less than about 1% of the total weight of the grain which constitutes at least a portion of the batch.

7. Ceramically bonded basic refractory shapes suitable for use in metallurgical vessels, said shapes, by weight and on the basis of an oxide analysis, consisting essentially of from about 0.8 to no more than about 1% SiO<sub>2</sub>, CaO in an amount sufficient to obtain a CaO to SiO<sub>2</sub> weight ratio between about 3 to 1 and about 4 to 1, the remainder consisting essentially of MgO and materials of the group Fe<sub>2</sub>O<sub>3</sub>, Cr<sub>2</sub>O<sub>3</sub>, and Al<sub>2</sub>O<sub>3</sub>, said latter materials constituting less than about 1% of the total weight of the batch.

8. Ceramically bonded basic refractory shapes made from a batch of size graded refractory grain consisting essentially of from about 0.8 to no more than about 1% SiO<sub>2</sub>, CaO in an amount sufficient to obtain a CaO to SiO<sub>2</sub> weight ratio between about 3 to 1 and about 4 to 1, the remainder consisting essentially of MgO and materials of the group Fe<sub>2</sub>O<sub>3</sub>, Cr<sub>2</sub>O<sub>3</sub>, and Al<sub>2</sub>O<sub>3</sub>, said latter materials constituting less than about 1% of the total weight of the batch.

9. Ceramically bonded basic refractory shapes suitable for use in metallurgical vessels, said shapes made from a batch of size graded dead burned magnesia grain, at least a portion of the grain, by weight and on the basis of an

oxide analysis, consisting essentially of from about 0.8 to no more than about 1% SiO<sub>2</sub>, CaO in an amount sufficient to obtain a CaO to SiO<sub>2</sub> weight ratio between about 3 to 1 and about 4 to 1, the remainder consisting essentially of MgO and materials of the group Fe<sub>2</sub>O<sub>3</sub>, Cr<sub>2</sub>O<sub>3</sub>, 5 and Al<sub>2</sub>O<sub>3</sub>, said latter materials constituting less than about 1% of the total weight of the batch.

## References Cited in the file of this patent

## UNITED STATES PATENTS

3,106,475 Davies et al. ----- Oct. 8, 1963

## OTHER REFERENCES

Holt, J.: "Tar Bonds Oxygen Vessel Bricks," in Steel, vol. 143, pp. 74-78, July 7, 1958, TS 300 174, 266-43.

UNITED STATES PATENT OFFICE  
CERTIFICATE OF CORRECTION

Patent No. 3,141,790

July 21, 1964

Ben Davies et al.

It is hereby certified that error appears in the above numbered patent requiring correction and that the said Letters Patent should read as corrected below.

Column 9, line 7, after "weight" insert -- of the grain  
which constitutes at least a portion --.

Signed and sealed this 12th day of January 1965.

(SEAL)

Attest:

ERNEST W. SWIDER  
Attesting Officer

EDWARD J. BRENNER  
Commissioner of Patents